# EUROPEAN PATENT SPECIFICATION

(11) **EP 1 379 702 B1**
(45) Date of publication and mention of the grant of the patent: **10.08.2005**
(21) Application number: 01967378.9
(22) Date of filing: 12.09.2001
(51) Int. Cl.: C21D 1/06, C21D 9/36

(54) **METHOD FOR MAKING A ROLL SHELL OF A ROLL USED IN THE MANUFACTURE OR FURTHER PROCESSING OF PAPER AND/OR BOARD**
VERFAHREN ZUR HERSTELLUNG EINES WALZENMANTELS EINER BEI DER HERSTELLUNG ODER WEITERVERARBEITUNG VON PAPIER UND/ODER PAPPE VERWENDETEN WALZE
PROCEDE DE FABRICATION D'UNE VIROLE D'UN CYLINDRE UTILISE DANS LA FABRICATION OU LE TRAITEMENT DU PAPIER ET/OU DU CARTON

(30) Priority: 15.09.2000 FI 20002045
(43) Date of publication of application: 14.01.2004
(73) Proprietor: Metso Paper, Inc., 00130 Helsinki (FI)
(72) Inventor: BLOMSTER, Kari, FIN-02320 Espoo (FI)
(74) Representative: Leson, Thomas Johannes Alois, Dipl.-Ing.
(86) International application number: PCT/FI2001/000792
(87) International publication number: WO 2002/024964

(56) References cited:
- GB-A- 906 029
- US-A- 4 444 556

## Description

The present invention relates to a method for making a roll shell and, more particularly, the invention relates to a method for making a roll shell of a heatable roll, i.e. a so-called thermo roll, which roll operates in practice as heated to a high temperature.

More specifically, the invention relates to a method for making a roll shell of a roll used in the manufacture or further processing of paper and/or board, in which method a shell blank of the roll shell is made of steel and the shell blank is subjected to heat treatments comprising heating for hardening, quenching and tempering treatments.

In prior art there is known a solution in which a wrought steel shell is subjected to surface hardening by means of induction. A considerable drawback with this is, however, that the method is remarkably expensive and, in addition, that long and large-diameter roll blanks cannot be hardened economically by induction. Surface hardening by induction requires that expensive ancillary equipment shall be arranged for the sole purpose of hardening. It has been necessary to separately provide large-diameter rolls which cannot be hardened economically by induction, for example, with a wear-resistant hard coating. If again it were contemplated that, for example, the quenching of a large-diameter roll blank is carried out into a water basin, both sides of the shell will undergo hardening and tensile stress will be created in the surface. Because of the risk of breakage, it is very harmful when tensile stress remains in the roll surface.

With respect to the state of the art, reference is further made, for example, to US patent *5,546,856* describing a paper finishing method in which a long nip calender is made use of. By a long nip calender is generally meant a calender in which a nip is formed between a heatable steel roll and a belt. The nip pressure in the long nip calender can be regulated in the cross direction of the machine, i.e. in the CD direction, whereby, for example, the thickness of paper can be profiled. The long nip calender can be formed of a belt calender in which a belt is passed, while guided by auxiliary rolls, around one nip roll serving as a backing roll for a thermo roll. Thus, the long nip is formed between the thermo roll and said nip roll loading the belt. The most common long nip calender is a shoe calender in which the belt is arranged to run around a stationary support structure and in which the belt is loaded against a thermo roll by means of a loading shoe which is located inside the loop of the belt and supported on the support structure. In the shoe calender, the long nip is formed between the thermo roll and the shoe loading the belt. Thus, the loading shoe of the shoe calender determines the length of the nip.

In the shoe calenders which represent the state of the art and which are in use, the length of the nip is typically in a range of 50-70 mm, i.e. the dwell time of the web in the nip is considerably below 10 ms. The surface temperature of the thermo roll serving as the backing roll of the shoe roll is in a range of 70-300 °C, and the maximum pressure of the nip is in a range of 5-10 MPa. The hardness of the calender belt in the shoe calender is in a range of 70-100 ShA. Longer nips of about 270 mm have been used in presses that are based on a shoe roll.

US 4 444 556 discloses a cooling apparatus, wherein a hot metal tube or the like axially travels along a path extending through cooling fluid shower nozzles for quenching or controlled cooling.

GB 906 029 discloses a method of quenching heated work-rolls of different shape by directing a quenching liquid onto and around the work-roll from an encircling quench unit so that the liquid flows down in the form of a sheath or stocking.

The method of making a roll according to the invention is not suitable for use in making rolls which are used in long nip calenders according to the state of the art.

The aim of the present invention is to provide a novel method for making a roll shell, which method allows drawbacks and problems associated with the state of the art to be avoided or at least substantially reduced. With a view to achieving this aim, the invention is characterized is carried out such that hardening takes place in a directed manner from the outer by the subject-matter of claim 1.

In accordance with the invention, a tubular shell of a thermo roll is made of an alloy steel, for example, of a quenching and tempering steel such that a wrought steel blank is first made which is heat-treated after that in a suitable manner in order to achieve desired properties. The heat treatment is carried out in a manner in which formation and decomposition of austenite occurs. The aim of the heat treatment is to provide the roll shell with a hard and wear-resistant surface so that the roll is suitable as such for use, for example, as a heatable roll in a calender. On the other hand, the surface produced and the basic structure of the material of the roll shall be such as to be suitable for being coated and/or uncoated. Further, the properties of the material of the roll after heat treatment shall be such that in the roll shell there are no harmful stresses, which might cause the roll to break as a result of abrupt temperature variations.

The roll shell according to the invention is manufactured of a well-hardening steel, for example, of a quenching and tempering alloy steel and, as one very usable grade, 34NiCrMo 6 steel is suitable for manufacture. The desired properties are attained such that, when the shell blank (steel blank) has been made, it is heat-treated such that the blank is subjected to heating for hardening to a high temperature above the temperature of formation of austenite, to a range of about 820-920 °C. The quenching of the blank is performed after that in order to harden the blank, i.e. to form martensite in the structure. The quenching is carried out into a medium, for example, in a basin. The medium can be a liquid, for example, water or a liquid mixture, a gas mixture or a combination of a liquid and a gas mixture. The quenching can also be carried out by a fluidized bed method. It is essential that before quenching the ends of the shell blank are closed, or water or another quenching medium is prevented by some other means from getting into the interior of the blank, to the inner surface of the blank. This provides the benefit that in connection with quenching, hardening, i.e. formation of martensite begins only from the outer surface of the shell blank, from which cooling proceeds in a directed manner in the material inwards. Consequently, in the invention, the inner parts of the roll material are not hardened, as a rule, completely at any rate. When in the invention, for example, the through hardening of the wall of the material is inhibited, the wear resistance of the roll material is improved. Tempering and relieving of residual stresses can be carried out after quenching. When manufactured according to the method of the invention, the roll shell is made metallurgically very stable. If the invention is intended particularly for the manufacture of a thermo roll shell, the shell shall be additionally provided with perforations for circulation of a heating medium. These holes or axial bores can be formed in the roll shell either before hardening or after hardening.

Thus, the change of the microstructure of the material from a martensitic structure to a bainitic or a bainitic-martensitic or a bainitic-ferritic structure or to combinations of them occurs steplessly. This enables neutral or compression stress to be formed advantageously in the outer surface of the shell from which cooling begins, because with the progress of cooling the increase in the volume of material becomes smaller in the direction from the surface towards the interior. Since a neutral stress state or compression stress is created in the outer surface, the shell is not prone to damage or breakage even when abrupt variations of temperature occur in a finished roll which is in use. Such variations are possible if, for example, a liquid, e.g. water, is passed to a hot roll surface. If tensile stress remained in the surface, rapid cooling of a hot roll might cause the roll to break. The formation of tensile stress in the surface of the roll is prevented by means of the invention.

In the following, one method of making a roll shell is described by way of example.

The steel used as material:
- DIN 34NiCrMo 6, number identification 1.6582

### Analysis:

- C% 0.30-0.38, Si% ≤ 0.4, Mn% 0.5-0.8, P% <0.035, S% ≤ 0.035, Cr% 1.3-1.7, Mo% 0.15-0.30, Ni% 1.3-1.7

### Mechanical values:

- Tensile strength 1000-1200 N/mm²
- Elongation from a transversely taken tension test bar ≤ 12%
- Hardness 350-500 HV₂₀
- Heat resistance 300 °C about -15%

### Microstructure in the surface:

- 100% tempered martensite

The melting of steel takes place in an electric arc furnace (EAF) and the alloying proper as well as the setting of temperature take place in a holding furnace (LF), which is provided with electromagnetic stirring. Casting is carried out by up-running casting into an ingot mould. When the casting has solidified and cooled to about 600 °C, it is moved to a forge, into a heating furnace in which it is heated to a temperature of about 1200-1285 °C at which forging is started and which is the temperature of the furnace.

The roll shell (tube) is made out of the casting by forging as a free forging. Advantageously, a sturdy hydraulic press is employed in forging, which makes it possible to use sturdy tools, by means of which the low density in the middle of the casting can be compressed. In a tubular forging, the low density portion in the middle is cut off so as to form a blank for a centre hole to be made. Slag materials and other defects collected in the casting are removed from the cast mass in connection with forging. The manufacture of a tubular forging takes place by pressing on a mandrel. When forged in the manner described above, the degree of deformation of the roll tube can be made uniformly good.

After forging, heat treatments are carried out such that there is first cooling in the air. This is immediately followed by normalizing to 820-920 °C, from which cooling takes place freely into the air. Immediately after that, soft annealing is carried out at about 630-700 °C, which is followed by cooling to room temperature. The thus heat-treated steel is fine-grained, soft annealed for a quenching and tempering treatment.

Since the surface of the blank must become clean, the blank is subjected to rough machining before it is quenched and tempered to a desired strength/hardness level. In that connection, soft annealing is of advantage because normally a large amount of material has to be removed. Quenching and tempering, i.e. heating to the austenite range and tempering after hardening are carried out in a furnace. The quenching can be carried out into a liquid basin, for example, into an oil basin or water basin, or quenching can be carried out as air quenching. Since the strength level requirements of the piece are high, it is advantageous that the roll shell blanks are quenched into water. Tempering is carried out immediately after quenching at a temperature of about 340-660 °C. Since it is a question of making a roll shell of a so-called thermo roll, the shell shall be provided further with substantially axial peripheral bores for circulation of a heating medium in the finished roll. These peripheral bores can be made when the shell is in a quenched and tempered state.

The invention is not strictly confined to the description given above nor to the specific mode of operation of the invention set forth in the description, but the different modes of operation of the invention may vary within the inventive idea defined in the accompanying claims.

## Claims

1. A method for making a roll shell of a roll used in the manufacture or further processing of paper and/or board, in which method a shell blank of the roll shell is made of steel and the shell blank is subjected to heat treatments comprising heating for hardening, quenching and tempering treatments, wherein the quenching is carried out such that hardening takes place in a directed manner from the outer surface of the roll shell inwards, **characterised in that** the quenching is carried out by means of a fluidised bed method, wherein the quenching medium is prevented from getting to the inner surface of the roll shell.

2. A method according to claim 1, **characterised in that** the quenching is carried out such that neutral or compression stress is produced in the surface of the roll.

3. A method according to any one of the preceding claims, **characterised in that** the formation of tensile stress in the surface if the roll is prevented by quenching.

4. A method according to any one of the preceding claims, **characterised in that** the roll shell is provided with through holes or equivalent bores extending mainly in the axial direction before heat treatment or after heat treatment.

## Patentansprüche

1. Verfahren zur Herstellung eines Walzenmantels einer Walze, die in der Herstellung oder weiteren Bearbeitung von Papier und/oder Pappe verwendet wird, in welchem Verfahren ein Walzenrohling des Walzenmantels aus Stahl hergestellt wird, und der Walzenmantel Wärmebehandlungen unterzogen wird, welche Aufheizen zum Härten, Abschrecken und Temperbehandlungen umfassen, wobei das Abschrecken in einer solchen Art und Weise ausgeführt wird, daß das Härten in einer gerichteten Art und Weise von der äußeren Oberfläche des Walzenmantels nach innen ausgeführt wird,
**dadurch gekennzeichnet, daß**
das Abschrecken mit Hilfe eines Fluidbettverfahrens ausgeführt wird, wobei das Abschreckmedium daran gehindert wird, auf die innere Oberfläche des Walzenmantels zu gelangen.

2. Verfahren nach Anspruch 1, **dadurch gekennzeichnet, daß** das Abschrecken so ausgeführt wird, daß neutrale Spannungen oder Druckspannungen in der Oberfläche der Walze erzeugt werden.

3. Verfahren nach einem der vorhergehenden Ansprüche, **dadurch gekennzeichnet, daß** die Bildung von Zugspannung in der Oberfläche der Walze durch Abschrecken verhindert wird.

4. Verfahren nach einem der vorhergehenden Ansprüche, **dadurch gekennzeichnet, daß** der Walzenmantel vor der Wärmebehandlung oder nach der Wärmebehandlung mit durchgängigen Löchern oder äquivalenten Bohrungen versehen wird, welche sich hauptsächlich in der axialen Richtung erstrecken.

## Revendications

1. Procédé de fabrication d'une virole d'un rouleau utilisé dans la fabrication ou le traitement supplémentaire de papier et/ou de carton, dans lequel procédé une ébauche de la virole est faite en acier, et l'ébauche est soumise à des traitements à chaud comprenant des traitements de chauffage pour durcissement, de refroidissement et de trempe, dans lequel le refroidissement est exécuté de telle sorte que le durcissement se fasse d'une manière dirigée depuis la surface extérieure de la virole vers l'intérieur, **caractérisé en ce que** le refroidissement est exécuté selon un procédé à lit fluidisé dans lequel le milieu de refroidissement est empêché d'atteindre la surface intérieure de la virole.

2. Procédé selon la revendication 1, **caractérisé en ce que** le refroidissement est exécuté de telle sorte qu'une contrainte neutre ou de compression se produise sur la surface du rouleau.

3. Procédé selon l'une quelconque des revendications précédentes, **caractérisé en ce que** la formation d'une contrainte de tension sur la surface du rouleau est empêchée par refroidissement.

4. Procédé selon l'une quelconque des revendications précédentes, **caractérisé en ce que** la virole est percée de trous de passage ou d'orifices équivalents s'étendant principalement dans la direction axiale avant le traitement à chaud ou après le traitement à chaud.
